# EUROPEAN PATENT SPECIFICATION

(11) **EP 0 064 295 B1**
(45) Date of publication and mention of the grant of the patent: **21.11.1985**
(21) Application number: 82103813.0
(22) Date of filing: 04.05.1982
(51) Int. Cl.: C23F 11/00, C23F 17/00, C23F 1/00, C23F 1/20, C23G 1/12

(54) **Method of improving the corrosion resistance of chemical conversion coated aluminum**
Verfahren zur Verbesserung des Korrosionswiderstandes von durch chemische Umwandlung beschichtetem Aluminium
Procédé pour l'amélioration de la résistance à la corrosion d'aluminium enduit par conversion chimique

(30) Priority: 04.05.1981 US 260370
(43) Date of publication of application: 10.11.1982
(73) Proprietor: Batiuk, Walter, Seattle Washington 98105 (US)
(72) Inventor: Batiuk, Walter, Seattle Washington 98105 (US)
(74) Representative: Hoijtink, Reinoud

## Description

The invention relates to a method for treating aluminum to enhance corrosion resistance of its surface, which includes deoxidizing the aluminum surface with deoxidizing means and coating the aluminum surface with a chemical conversion solution.

Conversion coated aluminum has been used by airframe and other manufacturers, including the military, to improve aluminum's corrosion resistance and paint adhesion properties. In the prior art, the aluminum is deoxidized using a chromated deoxidizer, and then coated in the conversion process with a coating resistant to corrosion. When coated aluminum is manufactured for use in military applications, a stringent corrosion resistant test must be met as outlined in Military Specification MIL-C-5541 and MIL-C-81706. These tests require subjecting the finished aluminum product to a salt spray for a lengthy period of time, such as 164 to 328 hours, respectively.

Prior to the present invention, it was extremely difficult to pass the salt spray requirement imposed by the military for aluminum hardware. Special conversion coatings were developed, and various deoxidizers used. In general, the aluminum was treated using a chromated deoxidizer to etch away the natural and heat-treat oxide so that the finished product has a uniform color and texture. A chemical conversion coating is applied to the aluminum. One typical coating is "Alodine 1200S" manufactured by the Amchem Products, Inc., Ambler, PA. This conversion coating consists of a corrosion resistant brown irridescent layer. This film has potential good resistance to normal corrosion; however, in highly corrosive environments such as that required by the salt spray test, the film may succumb to corrosion and not meet military specifications. In general, the prior art relied upon chromated deoxidizers to meet the stringent corrosion requirement tests. Non-chromated deoxidizers were tested, but failed to meet the military specification requirements after being chemically conversion coated. Deoxidizers containing the chromate ion, although producing better results in salt spray test requirements, have a pollution problem due to the effluent stream. Heavy metals, such as chrome, are highly toxic to the environment, and are therefore undesirable for release into closed or open bodies of water. Previous to the present invention, a workable non-chromated treatment process prior to chemical conversion coating aluminum was lacking if salt spray requirements were to be consistently met.

The U.S. Patent No. 2,351,465 issued to Watcher deals with the use of sodium nitrite as an inhibitor to corrosion inside steel pipelines carrying petroleum distillates. This invention, specifically, needed to protect the pipelines from distillates containing hydrocarbon oils; and not salt spray as the present invention. Ferguson, in U.S. Patent No. 2,671,717 teaches the use of sodium nitrate in brightening aluminum, not for corrosion resistance.

A non-chromated deoxidizer is disclosed in U.S. Patent No. 3,140,203 issued to Grunwald; however, this patent does not teach the applicability and compatability of this deoxidizer with a conversion coating. U.S. Patent No. 3,275,562, issued to Smith, shows one formulation of a non-chromated aluminum de-smutter. Hatch, in U.S. Patent No. 3,335,096, deals with a corrosion protective chemical in a closed system which protects the metal surface only while in contact with the surface. As in the previously cited U.S. patent, Thornhill (U.S. patent No. 3,340,001) teaches a composition for protecting metal from corrosion which is constantly in contact with the metal. This composition contains sodium nitrite; however, it is not obvious from Thornhill that this composition would have good results when combined with chemical conversion coating. Shick, in U.S. Patent No. 3,433,577, uses a composition containing sodium nitrite for protecting metal parts from corrosion. The purpose of this composition is for vapor phase corrosion inhibitors during storage, but does not indicate the applicability for enhancing the corrosion resistance to salt spraying. U.S. Patent No. 3,445,400 issued to Everhart contains a chromated formulation. Bland et al, in U.S. Patent No. 3,510,430 discloses a ferric sulfate non-chromated deoxidizer which would not satisfactorily meet salt spray tests. The nitrates in this formulation are used to prevent pitting during deoxidization. U.S. Patent No. 3,802,973 teaches an oxidizing agent to uniformly etch aluminum in an alkaline solution for the purpose of hiding surface defects.

The present invention discloses a method for treating aluminum metal to enhance corrosion resistance of its surface, which includes deoxidizing the aluminium surface with deoxidizing means and coating the aluminium surface with a chemical conversion solution.

The method is characterized by exposing the aluminum surface deoxidized with said deoxidizing means to a nitrite solution having a pH below 5, before conversion coating with said chemical conversion solution.

In order to provide a method for treating aluminum which eliminates an effluent stream containing chromate, it is preferred, that said deoxidizing means is a non-chromated deoxidizer, preferably said non-chromated deoxidizer is a nitric acid solution with a concentration of nitric acid of at least 10%, preferably 15% to 25%, by volume based on 10% nitric acid. In another preferred embodiment said non-chromated deoxidizer is a nitric acid solution with a concentration of nitric acid of 30%-50% based on commercial grade nitric acid.

In a preferred embodiment of the invention a fluoride iron is present in said deoxidizing nitric acid solution since the fluoride iron is one of the best etching agents of unfinished aluminum metal, and can etch uniformly without pitting. Therefore it is preferred, that said nitric acid solution contains a sufficient concentration of fluoride iron to etch the aluminum surface at a rate of at least 0.00125 mm/hr (0,05 mils/hr). Supplement to the etching action of the fluoride iron, nitric acid is used to remove undissolved silicon from the aluminum surface and to prevent the formation of smut which is a redeposit of copper.

The treatment with the nitrite solution is especially effective if said nitrite solution is maintained at a pH of 3 or less.

It is preferred that said nitrite solution is substantially contributed by sodium nitrite, potassium nitrite and/or a mixture of sodium and potassium nitrite.

The best results to enhance the corrosion resistance of the aluminum surface are achieved, by drying said aluminum the surface of which is coated with said chemical conversion solution, at a temperature between 43°C (110°F) and 54°C (130°F). The present invention may be practiced on the following sequence of operation:
1) vapor degreasing the aluminum;
2) alkaline cleaning the aluminum;
3) rinsing the aluminum with water;
4) deoxidizing the aluminum, preferably with a non-chromated deoxidizer;
5) rinsing the deoxidized aluminum with water;
6) exposing the aluminum to a sodium nitrite solution;
7) rinsing the aluminum with water;
8) chemical conversion coating the aluminum; and
9) drying the aluminum.

Vapor degreasing of the aluminum metal can be performed by standard techniques known to one skilled in the art. Similarly, alkaline cleaning and rinsing of the aluminum are steps commonly known to those skilled in the art and insure a clean aluminum surface prior to deoxidization.

The deoxidization step which is the next step is preferably produced with a non-chromated deoxidizer. A chromated deoxidizer is undesirable from a pollution standpoint since chrome or chrome ions are toxic, and the effluent stream may be released to open bodies of water. The invention can be practiced, however, using a chromated deoxidizer if desired and the resulting product will readily meet the salt spray requirements of the military.

Other non-chromated deoxidizers may be used in the practice of the invention without losing the beneficial effects of treating aluminum in the manner taught by the inventor. The aluminum may be immersed in the deoxidizer for approximately 5 minutes to 60 minutes or greater, depending on the difficulty of scale removal. The nitric acid deoxidizer performs best when a freshly prepared solution is buffered with some dissolved metallic aluminum.

After deoxidization, the aluminum is then rinsed with cold water, and a supplemental treatment, differing from the prior art, is performed to allow the final conversion coated product to pass salt spray requirements. In this step, the deoxidized aluminum is rinsed with a sodium nitrite solution. The aluminum may either be immersed in the solution or sprayed with the solution. The sodium nitrite solution is maintained at a pH less than 5 and preferably at pH 3 or below. Nitric acid can supply the necessary hydrogen ion concentration. The concentration of sodium nitrite is not critical, assuming the pH is less than 5, and beneficial results can be obtained with a sodium nitrite solution of 1%. After the sodium nitrite treatment, a water rinse of the aluminum is performed prior to chemical conversion coating. It should also be noted that potassium nitrite may be used in place of sodium nitrite with beneficial results.

The chemical conversion coating can be done with any of the coating solutions known to the prior art. It has been found that Alodine 1200S, manufactured by Amchem Products, Inc., Ambler, PA, works satisfactorily.

To coat the aluminum, immersion in the coating solution is allowed to take place for a relatively short time such as up to five minutes.

After conversion coating, the aluminum is dried by warm air. In the preferred embodiment of the invention, the drying temperature will be in the range of 43°C (110°F) to 54°C (130°F) with an optimum at 49°C (120°F). The present invention may be further understood by reference to the following examples and accompanying tables.

### Example 1

B are aluminum alloy specimens 25.4 cm by 7.6 cm (10" by 3") were used in this and all other examples. Table 1 shows the results of this series of samples which illustrates the effect of sodium nitrite treatment on the salt spray test results. A partially depleted chromate-type deoxidizer was used called Am Chem 6-17, a product of Amchem Products, Inc., Ambler, PA. As in all examples, each specimen was first cleaned using an alkaline cleaner called Turco 2623, a product of the Turco Products Division of Purex Corporation Ltd., Wilmington, California. The alkaline cleaning was conducted for 30 minutes at 60°C (140°F). Deoxidation occurred in Amchem 6-17 with the etch rate adjusted to 0.0064 mm/side/hr (0.25 mils/side/hr) with hydrogen fluoride. The next processing step for the bottom four specimens on Table 1 was an immersion in the sodium nitrite solution for 30 minutes. The solution had a pH of 3 and a concentration of 3%. The top four specimens did not receive a sodium nitrite immersion. All specimens were then immersed in Alodine 1200S and dried for 30 minutes at a temperature of 43°C-54°C (110°F-130°F). It should be noted that all specimens in all examples were rinsed with tap water after each processing step.

Table 1 shows that only the specimens which were immersed in the sodium nitrite solution passed the salt spray test, i.e. the top four specimens of Table 1 had one or more corrosion pits visible to the unaided eye, indicating failure, while the bottom four specimens had no visible corrosion pits, indicating passing results.

In this example, as in all other examples, the tests were concluded after one week of salt spray immersion for visual examination and other evaluation tests.

### Example 2

Bare alloy specimens similar to those used in Example 1 were used in Example 2. The main difference in the two examples was the use of a non-chromated ferrous ion-type deoxidizer instead of a chromated deoxidizer. The deoxidizer in this example was Isoprep 184, a product of Allied-Kelite Products Division, Los Angeles, California. It was used in a 25% concentration with an etch rate of 0.0064 mm/side/hr (0.25 mils/side/hr) maintained with hydrogen fluoride addition. The sodium nitrite solution was 2.3% sodium nitrite with a pH of 3.0. This example illustrates that the only specimens which passed the salt spray test (no pits visible to the unaided eye) were those immersed in the sodium nitrite solution see Table 2).

### Example 3

Example 3 is similar to Examples 1 and 2, differing only in the deoxidizer used. In Example 3, a nitric acid-fluoride ion type non-chromate deoxidizer was used. The specimens were processed in the same manner as Examples 1 and 2. The deoxidizer consisted of 40% by volume of concentrated nitric acid (technical grade) with a sufficient fluoride ion concentration to produce an etch rate of 0.0064 mm/side/hr (0.25 mils/side/hr). The sodium nitrite solution was of a 2.3% concentration with a pH of 3.3. The results outlined in table 3 show that the specimens passing the salt spray test were those which were immersed in sodium nitrite. The specimens which were not immersed in the sodium nitrite solution failed the test.

### Example 4

In Example 4, a nitric acid-fluoride ion type non-chromated deoxidizer was used as in Example 3. Instead of immersion in a sodium nitrite solution after this processing step, a potassium nitrite solution of 2.3% concentration with a 3.0 pH was used. The results in Table 4 show that the specimens which were not immersed in the potassium nitrite solution failed to pass the salt spray test. The specimens that were immersed in potassium nitrite, however, passed the salt spray test.

### Example 5

Example 5 uses Isoprep 184, a ferrous ion-type non-chromated deoxidizer as did Example 2. Instead of sodium nitrite, potassium nitrite was used in the next processing step. The solution was of 2.3% concentration with a pH of 3.0. As seen in Table 5, the only specimens passed were those treated with potassium nitrite.

## Claims

1. Method for treating aluminum to enhance corrosion resistance of its surface, which includes deoxidizing the aluminum surface with deoxidizing means and coating the aluminum surface with a chemical conversion solution; characterized by exposing the aluminum surface deoxidized with said deoxidizing means to a nitrite solution having a pH below 5, before conversion coating with said chemical conversion solution.

2. Method as claimed in claim 1, characterized in that said deoxidizing means is a non-chromated deoxidizer.

3. Method as claimed in claim 2, characterized in that said non-chromated deoxidizer is a nitric acid solution with a concentration of nitric acid of at least 10% by volume based on 100% nitric acid.

4. Method as claimed in claim 3, characterized in that said concentration of nitric acid is 15%-25% by volume.

5. Method as claimed in claim 2, characterized in that said non-chromated deoxidizer is a nitric acid solution with a concentration of nitric acid is 30%-50% based on commercial grade nitric acid.

6. Method as claimed in claim 3, 4, or 5, characterized in that said nitric acid solution contains a sufficient concentration of fluoride ion to etch the aluminum surface at a rate of at least 0.00125 mm/hr (0.05 mils/hr).

7. Method as claimed in any of the preceding claims, characterized in that the pH of said nitrite solution is 3 or less.

8. Method as claimed in any of the preceding claims, characterized in that said nitrite solution is substantially contributed by sodium nitrite.

9. Method as claimed in any of the preceding claims 1-7, characterized in that said nitrite solution is substantially contributed by potassium nitrite.

10. Method as claimed in any of the preceding claims 1-7, characterized in that said nitrite solution is substantially contributed by a mixture of sodium and potassium nitrite.

11. Method as claimed in any of the preceding claims, characterized by drying said aluminum the surface of which is coated with said chemical conversion solution, at a temperature between 43°C (110°F) and 54°C (130°F).

## Patentansprüche

1. Verfahren zur Behandlung von Aluminium zwecks Verbesserung des Korrosionswiderstandes auf der Oberfläche, welches folgende Schritte umfaßt es wird die Aluminiumoberfläche mit einem Desoxydationsmittel desoxydiert und es wird die Aluminiumoberfläche mit einer chemischen Umwandlungslösung überzogen, dadurch gekennzeichnet, daß die durch das Desoxydationsmittel desoxydierte Aluminiumoberfläche einer salpetrigsauren Lösung ausgesetzt wird, die einen pH-Wert unter 5 besitzt, bevor der Umwandlungsüberzug mit der chemischen Umwandlungslösung aufgetragen wird.

2. Verfahren nach Anspruch 1, dadurch gekennzeichnet, daß das Desoxydationsmittel ein chromfreies Desoxydationsmittel ist.

3. Verfahren nach Anspruch 2, dadurch gekennzeichnet, daß das chromfreie Desoxydationsmittel eine Salpetersäure-Lösung mit einer Konzentration von Saltpetersäure von wenigstens 10 Volumenprozent ist, basierend auf einer 100%-igen Salpetersäure.

4. Verfahren nach Anspruch 3, dadurch gekennzeichnet, daß die Konzentration der Saltpetersäure 15-25 Volumenprozent beträgt.

5. Verfahren nach Anspruch 2, dadurch gekennzeichnet, daß das chromfreie Desoxydationsmittel eine Saltpetersäure-Lösung mit einer Konzentration von Saltpetersäure von 30%-50% ist, basierend auf einer kommerziellen Klasse einer Salpetersäure.

6. Verfahren nach den Ansprüchen 3,4 oder 5, dadurch gekennzeichnet, daß die Salpetersäure-Lösung eine ausreichende Konzentration von Fluorid-lonen enthält, um die Aluminiumoberfläche mit einer Geschwindigkeit von wenigstens 0,00125 mm/h (0,05 mils/h) zu ätzen.

7. Verfahren nach einem der vorhergehenden Ansprüche, dadurch gekennzeichnet, daß der pH-Wert der salpetrigsauren Lösung 3 oder weniger beträgt.

8. Verfahren nach einem der vorhergehenden Ansprüche, dadurch gekennzeichnet, daß die salpetrigsaure Lösung im wesentlichen von Natriumnitrit gebildet ist.

9. Verfahren nach einem der vorhergehenden Ansprüche 1 bis 7, dadurch gekennzeichnet, daß die salpetrigsaure Lösung im wesentlichen von Kaliumnitrit gebildet ist.

10. Verfahren nach einem der vorhergehenden Ansprüche 1 bis 7, dadurch gekennzeichnet, daß die salpetrigsaure Lösung im wesentlichen von einer Mischung aus Natriumnitrit und Kaliumnitrit gebildet ist.

11. Verfahren nach einem der vorhergehenden Ansprüche, dadurch gekennzeichnet, daß die Oberfläche des Aluminiums, die mit der chemischen Umwandlungslösung überzogen wird, bei einer Temperatur zwischen 43°C (110°F) und 54°C (130°F) getrocknet wird.

## Revendications

1. Procédé de traitement de l'aluminium pour augmenter la résistance à la corrosion de sa surface, qui comprend la désoxydation de la surface de l'aluminium avec des moyens désoxydants et le revêtement de la surface d'aluminium avec une solution de conversion chimique; caractérisé en ce que l'on expose la surface d'aluminium désoxydée avec lesdits moyens désoxydants à une solution de nitrite ayant un pH inférieur à 5, avant le revêtement de conversion avec ladite solution de conversion chimique.

2. Procédé selon la revendication 1 caractérisé en ce que lesdits moyens désoxydants sont constitués par un désoxydant non chromaté.

3. Procédé selon la revendication 2 caractérisé en ce que ledit désoxydant non chromaté est une solution d'acide nitrique ayant une concentration d'acide nitrique d'au moins 10% en volume par rapport à de l'acide nitrique à 100%.

4. Procédé selon la revendication 3 caractérisé en ce que ladite concentration d'acide nitrique est de 15-25% en volume.

5. Procédé selon la revendication 2 caractérisé en ce que ledit désoxydant non chromaté est une solution d'acide nitrique ayant une concentration d'acide nitrique de 30-50% par rapport à de l'acide nitrique du commerce.

6. Procédé selon l'une quelconque des revendications 3, 4 ou 5 caractérisé en ce que ladite solution d'acide nitrique contient une concentration suffisante d'ion fluorure pour décaper la surface d'aluminium à une vitesse d'au moins 0,00125 mm/h.

7. Procédé selon l'une quelconque des revendications précédentes caractérisé en ce que le pH de ladite solution nitrique est de 3 ou moins.

8. Procédé selon l'une quelconque des revendications précédentes caractérisé en ce que ladite solution de nitrite est pratiquement obtenue à partir de nitrite de sodium.

9. Procédé selon l'une quelconque des revendications 1 à 7 caractérisé en ce que ladite solution de nitrite est pratiquement obtenue à partir de nitrite de potassium.

10. Procédé selon l'une quelconque des revendications 1 à 7 caractérisé en ce que ladite solution de nitrite est pratiquement obtenue à partir d'un mélange de nitrite de sodium et de potassium.

11. Procédé selon l'une quelconque des revendications précédentes caractérisé par un séchage dudit aluminium dont la surface est revêtue avec ladite solution de conversion chimique à une température entre 43-54°C.
